

[54] WIPING CLOTH

[75] Inventor: George Zeidell, San Diego, Calif.

[73] Assignee: International Clean Products, Inc.,  
San Diego, Calif.

[22] Filed: July 2, 1973

[21] Appl. No.: 375,837

## Related U.S. Application Data

[63] Continuation of Ser. No. 177,503, Sept. 2, 1971,  
abandoned.[52] U.S. Cl..... 53/21 FC; 15/208; 15/209 R;  
15/210 R; 8/137

[51] Int. Cl. .... B44d 1/092; D06m 13/02

[58] Field of Search ..... 117/138.8 B, 138.8 A,  
UA, 117/138.8 UA, 139.5 A, 139.5 CQ, 138.8 N,  
117/66, 47 R; 15/208, 209 R, 210 R;  
8/137, 137.5

## [56] References Cited

## UNITED STATES PATENTS

|           |         |                     |              |
|-----------|---------|---------------------|--------------|
| 2,693,427 | 11/1954 | Kingsford.....      | 117/138.8 N  |
| 2,974,432 | 4/1961  | Warnock et al. .... | 117/47 A     |
| 3,065,110 | 11/1962 | Hagge et al. ....   | 117/139.5 CQ |

|           |         |                      |              |
|-----------|---------|----------------------|--------------|
| 3,353,993 | 11/1967 | Kida et al.....      | 117/139.5 CQ |
| 3,424,609 | 1/1969  | Carl et al. ....     | 117/139.5 CQ |
| 3,459,697 | 8/1969  | Goldberg et al. .... | 117/138.8 N  |

Primary Examiner—William R. Trenor  
Attorney, Agent, or Firm—Brown & Martin

[57]

## ABSTRACT

Preparing a cloth of synthetic material for wiping, by washing the material in small quantities of a solution of hot filtered water and detergent at about 175° for about ten minutes, which solution comprises water filtered to about 5 micron filter to remove lint and to which is added about 3 ounces of detergent for about each 50 pounds of cloth to be washed; then rinsing the cloth in two rinses in water and thereafter in two hot water rinses to remove the detergent and unwanted lint; then rinsing the cloth in a cold water rinse and then in an antistatic solution for about 5 minutes, which antistatic solution comprises about 50% of water and 50% antistatic solution; and then rinsing the cloth in a cold water rinse, extracting the water from the cloth and placing the cloth in a plastic container.

1 Claim, No Drawings

## WIPING CLOTH

This is a continuation of application, Ser. No. 177,503, filed September 2, 1971, now abandoned.

## BACKGROUND OF THE INVENTION

## 1. Field of the Invention

This invention relates to wiping cloths and more particularly to a novel and improved wiping cloth and the method of processing the cloth so that it is clean, lint free and virtually free of contaminations and static electricity and the like.

## 2. Discussion of the Prior Art

There is a relatively large requirement for rags and other fabrics for wiping and cleaning purposes. Various 15 industrial institutions, shops, plants, garages and the like have a need for such cloths. Heretofore, these wiping cloths have been comprised of rags which are normally comprised of old clothing and the like, which are no longer useful for their intended purpose and have been previously discarded. These rags are, in most cases, washed and baled and thereafter resold to the industry for use in wiping and cleaning.

Oftentimes the need is for rags and cloths which are lint free and also free of any abrasives. In order to obtain a cloth or rag which is lint free and free of abrasives, it should also be one which will not attract lint and other contaminations and abrasives, it should be one which is free from any static electricity which will attract these contaminations into the rag or cloth.

This need is critical when used for cleaning delicate machinery such as hydraulic equipment on aircraft and the like. Should lint abrasives be introduced into these hydraulic systems by the contaminations of the wiping rags, the systems become clogged and fails to operate correctly. This failure in hydraulic systems becomes even more critical when considering the systems in aircrafts. Should the hydraulic systems in aircraft fail, the results are critical and oftentimes fatal.

Therefore, a need has arisen for a wiping cloth which meets certain standards, as to the amount of contaminants contained in a certain square footage of the rag.

## SUMMARY OF THE INVENTION

Briefly described, the present invention provides a wiping cloth comprised of a synthetic material such as Nylon, or the like, which is cut to its desired sizes. The cloths of synthetic material are then washed in a hot water solution containing a detergent mixture. The cloths are washed in small quantities in order to allow washing action to the highest degree. The temperature may be approximately 175° in one desired embodiment. The water, before being placed into the washing solution, is filtered, for example, in less than 5 micron count filter. A washing and rinsing cycle now takes place which includes an anti-static liquid formula which eliminates static electricity from the cloth. The solution is normally in the described embodiment 50 percent water and 50 percent anti-static solution. This anti-static solution follows the final cold water rinse. Thereafter, another extracting period commences to remove the detergent solution. The rags are then placed in a plastic container and then dried in a clean-room atmosphere.

This provides a cloth which is free of lint and other contaminations because of the fact that the cloth is comprised of a virtually lint free material. Thereafter,

the novel washing solution provided, in accordance with this invention, removes any further lint and contaminants from the cloth. The anti-static solution placed therein, then leaves the cloths in a condition, whereby, they will no longer attract further contaminations. When placed in the plastic bags, the cloths will remain in their uncontaminated condition until ready for use.

These and other features and advantages will become 10 more apparent to those skilled in the art, when taken into consideration with the following detailed description.

## DESCRIPTION OF ONE PREFERRED EMBODIMENT

In the processing of a cloth for the purpose of providing a lint free anti-static wiping cloth, it has been found that certain synthetic materials provide very little lint, that is, pieces of broken ends and gatherings of material 20 which break free or become disengaged from the material to which it is normally comprised. Because of the fact that synthetic materials are somewhat lint free, they make a very fine basis for the wiping cloths for use on critical hydraulic machinery and the like. These too 25 though, have been found to contain some lint and attract some contaminations and therefore, it is desired that these rags or cloths also be processed further to obtain a better result in its lint free use.

A cloth has been discovered which nearly meets the 30 criteria of the standards set down for wiping cloths and this is a nylon material manufactured under the trademark of 22N by Monsanto, having their general office in St. Louis, Missouri. These cloths are to some extent free from static-electrification. Other types of synthetic 35 materials which are virtually lint free may also be used, but it has been found that the best results of those tested, is with the 22N anti-static nylon by Monsanto.

It is possible to obtain cloth material from certain 40 types of milling and clothing manufacturing companies in the garment industries, whereby, the mill end cuts are available for sale. These mill end cuts can be obtained and processed in a manner hereinafter to be described. Also, of course, it is possible to directly purchase the cloth from the manufacturer or obtain them 45 in any other suitable manner. These special nylon cloths are then cut to the desired sizes and shapes, and thereafter washed in a solution hereinafter to be described.

The washing solution is generally a detergent in hot 50 water at about 175°F. It is found that 3 ounces of detergent for 50 lbs. of cloth is best suited. Any suitable detergent can be used. A detergent that can be used, for example, can be the type made by Philadelphia Quartz Company of California under the trademark of Score. 55 In one embodiment of this invention, it has been found that a 10 minute wash period in the above mentioned solution is sufficient with two 5 minutes rinses thereafter and two hot water 2 minute rinses for short extractions. Thereafter, a rinse in cold water of 3 minutes and a second rinse in cold water with 2 ounces of diluted anti-static solution is added thereto. The anti-static solution may be any suitable anti-static solution of which there are several, an example of one being Wallerstein AS20 manufactured by a division of Baxter Laboratory, Staten Island, New York. This solution of water soluble anti-static agent is diluted in 50 percent water and 60 50 percent anti-solution and is added to the final

rinse for 5 minutes. Thereafter, a third cold water 4 minute rinse extracting period is provided for the cloths. The cloths are then placed into a plastic container and dried in a clean room atmosphere.

It has been found that these special cloths processed in a solution in the above manner, will provide the ideal lint free anti-contaminated static-free cloths, which meets the criterion now needed in the industry and the governmental institutions in their plants to perform their wiping and cleaning criterion.

Having thus described one embodiment of this invention, what is claimed is:

1. The process of preparing a cloth of synthetic material for wiping purposes comprising the steps of, 10 filtering wash water through a 5 micron filter to remove lint, adding 3 ounces of detergent to the heated filtered wash water for 50 pounds of cloth to be washed in the wash water, washing cloths in small quantities in a solution of the 20

hot filtered water and detergent at about 175 degrees for a period of about 10 minutes, the synthetic material is nylon, rinsing the cloth in two 5 minute rinses in water and thereafter in two hot water 2 minute rinses to remove the detergent and unwanted lint, rinsing the cloths in cold water for a 3 minute rinse, rinsing the cloths in a second rinse in cold anti-static solution comprising 50 percent water and 50 percent anti-static solution for 5 minutes, rinsing the cloths in a third cold water 4 minute rinse and extracting the water from the cloths, placing the cloths in a plastic container and carrying the cloths to a clean room where the cloths are removed from the plastic container and dried in a clean room atmosphere, and then placing the cloths in a plastic container for storage until time of use.

\* \* \* \* \*